# EUROPEAN PATENT SPECIFICATION

(11) **EP 2 492 365 B1**
(45) Date of publication and mention of the grant of the patent: **11.12.2019**
(21) Application number: 11830869.1
(22) Date of filing: 04.10.2011
(51) Int. Cl.: C22C 23/04, C22C 23/02, C22C 23/00, C22C 23/06, C22C 1/02, C22C 1/03, B22D 21/04, C22F 1/06

(54) **FLAME RETARDANT MAGNESIUM ALLOY WITH EXCELLENT MECHANICAL PROPERTIES, AND PREPARATION METHOD THEREOF**
FEUERFESTE MAGNESIUMLEGIERUNG MIT HERVORRAGENDEN MECHANISCHEN EIGENSCHAFTEN UND HERSTELLUNGSVERFAHREN DAFÜR
ALLIAGE DE MAGNÉSIUM RETARDATEUR DE FLAMMES PRÉSENTANT D'EXCELLENTES PROPRIÉTÉS MÉCANIQUES ET PROCÉDÉ DE PRÉPARATION DE CELUI-CI

(30) Priority: 05.10.2010 KR 20100096709; 16.03.2011 KR 20110023260
(43) Date of publication of application: 29.08.2012
(73) Proprietor: Korea Institute Of Machinery & Materials, Daejeon 305-343 (KR)
(72) Inventor: KIM, Young Min, Changwon-si Gyeongsangnam-do 645-779 (KR); KIM, Ha Sik, Changwon-si Gyeongsangnam-do 630-511 (KR); YOU, Bong Sun, Changwon-si Gyeongsangnam-do 641 -766 (KR); YIM, Chang Dong, Changwon-si Gyeongsangnam-do 641-010 (KR)
(74) Representative: Patent- und Rechtsanwälte Ullrich & Naumann
(86) International application number: PCT/KR2011/007298
(87) International publication number: WO 2012/046984

(56) References cited:
- EP-A1- 1 048 743
- EP-A1- 1 777 022
- EP-A2- 1 526 188
- WO-A1-2006/075814
- CN-A- 101 037 753
- JP-A- H08 269 609
- JP-A- 2002 129 272
- JP-A- 2007 031 789
- JP-A- 2008 081 842
- JP-A- 2010 036 221
- JP-A- 2010 036 221
- KR-A- 20100 034 773
- US-A1- 2009 269 237

## Description

### [Technical Field]

The present invention relates to a magnesium alloy having excellent ignition resistance or nonflammability, and more particularly, to a magnesium alloy that can be melted and cast in the air as well as in a common inert atmosphere due to the presence of a stable protective film formed on the surface of the molten metal, has excellent ignition resistance or nonflammability in order to prevent spontaneous ignition of chips, and is excellent in both strength and ductility.

### [Background Art]

Magnesium alloys, which have a high specific strength, are the lightest of alloys, are applicable in a variety of casting and machining processes, and have a wide range of application, and are thereby used in almost all fields in which light weight is required, such as parts for vehicles and electronic parts. However, magnesium (Mg) is a metallic element that has a low electrochemical potential and is very active. Mg still has limitations in terms of the stability and reliability of the material, since it undergoes a strong reaction when it comes into contact with oxygen or water, and sometimes causes fires. Therefore, the fields in which Mg can be applied are still limited compared to its potential applicability. In particular, it cannot be used in applications in which safety is important.

Because of this activity of Mg alloys, it is necessary to create an inert atmosphere using an inert mixture gas, such as a flux or CO₂ + SF₆. Since the flux that is used in melting and refining is a chlorinated substance, there is a problem in that chlorine atoms reside inside a material, thereby significantly decreasing corrosion resistance when the conditions for processing the molten metal are not fulfilled. In order to solve this problem, it is effective to perform melting and casting in an atmosphere in which SF₆, CO₂ and air are mixed, instead of using the flux. However, SF₆ is classified as a greenhouse gas, the global-warming potential (GWP) of which is 24 times that of CO₂, so that the use thereof is expected to be regulated in the future time.

In order to more fundamentally solve this problem, studies for improving the oxidation resistance of Mg alloys, in particular, studies intended to increase the ignition temperature of Mg alloys by adding Ca, Be or rare-earth metals, have been carried out. Traditionally, Ca has been a main choice among the alloying elements that are added to Mg alloys that are oxidation resistant because Ca is cheaper than other rare-earth metals, is nontoxic, and greatly increases the ignition temperature in consideration of the amount that is added.

According to previous studies on magnesium alloys that contain Ca, it is known that the ignition temperature increases by about 250°C when 3wt% or greater of Ca is added. Therefore, in order to realize an ignition temperature of 700°C or higher, at which casting is possible in the condition of being exposed to the air without a protective gas, or an ignition temperature of 650°C or higher, at which casting is possible in the condition of including the protective gas, Ca must be added to Mg alloys, preferably in an amount of 3wt% or greater, and in a minimum amount of 2wt% or greater. However, when Ca is added in an amount greater than 2wt%, the tensile properties of Mg alloys are generally degraded, with the decrease in elongation being particularly significant. This is because a great quantity of coarse and brittle eutectic phases is formed, thereby resulting in cracks. As such, increasing the amount of Ca that is added has the merit of increasing the ignition resistance, but also has a drawback in that the tensile properties are significantly degraded. Therefore, there is the demand for the development of a magnesium alloy that can satisfy both the ignition resistance and the tensile properties.

WO 2006/075814 A1 relates to a wrought magnesium alloy comprising lanthanides (Group IIIa and Group IIIb) as an essential element that improves ductility and anisotropy and provides a wrought magnesium alloy which contains the intermetallic compound coherent to a matrix microstructure and which has a second phase composite microstructure, thereby improving elongation and anisotropy to assure excellent formability and corrosion resistance. WO 2006/075814 A1 is intended to solve the problem of greatly improving the moldability and corrosion resistance of magnesium alloys, but does not teach the description of a magnesium alloy having excellent ignition resistance and tensile properties at the same time.

JP 2010 036221 A relates to a flame-retardant magnesium alloy filler metal for obtaining high weld joint strength and preventing fume generation and further improving welding environment, which is composed of a flame-retardant magnesium alloy containing calcium as a base element. An object of the teaching of this document is to improve the welding environment by preventing the generation of fumes that become solid fine particles by cooling the material evaporated by heat during welding. This document teaches the flame-retardant magnesium alloy filler metal for obtaining high weld joint strength, which is composed of a flame-retardant magnesium alloy containing 0.5-5.0 mass% of calcium as a base element and one or more element chosen from boron (B), titanium (Ti), yttrium (Y), and zirconium as an additional additive (see Abstract of JP 2010 036221 A).

JP 2010 036221 A also teaches that the flame-retardant magnesium alloy filler metal is a magnesium alloy containing 0 to 12.0 wt% of aluminum, 0 to 5.0 wt% of zinc, and 0.5 wt% or less of manganese (see para [0018] of JP 2010 036221 A). However, JP 2010 036221 A does not teach that the ignition resistance of yttrium (Y) and its associated effects at all. JP 2010 036221 A provides the flame-retardant magnesium alloy filler metal having high weld joint strength and prevention of fume generation, but does not imply or teach the magnesium alloy having excellent ignition resistance and tensile properties at the same time.

### [Disclosure]

### [Technical Problem]

Therefore, an object of the present invention is to provide a magnesium alloy that is intended to solve the foregoing problem of the related art.

Specifically, an object of the present invention is to provide a magnesium alloy that contains Ca therein, and more particularly, has excellent ignition resistance and excellent tensile properties.

In addition, an object of the present invention is to provide a magnesium alloy that enables an environment-friendly manufacturing process, which uses a minimum amount of Ca and does not use a protective gas such as SF₆, which is an environmental pollutant.

### [Technical Solution]

In order to realize the foregoing object, according to the present invention, provided is a magnesium (Mg) alloy according to claim 1.

In addition, it is preferable that the content of the Ca range, by weight, from 0.2% to 1.5%.

Furthermore, it is preferable that the content of the Y range, by weight, from 0.1% to 1.5%.

In addition, it is preferable that the contents of the Ca and the Y range from 0.3% to 2.0% of a total weight of the magnesium alloy.

According to the present invention, provided is a method of manufacturing a magnesium alloy according to claim 5.

In addition, it is preferable that the step of adding the raw materials of Ca and Y into the magnesium alloy molten metal include the step of adding the raw materials of Ca and Y at a temperature higher than 800°C.

In addition, it is preferable that a master alloy ingot, which contains Mg, Al, Zn, Ca and Y, is soluble at 750°C or lower, and is input into the magnesium alloy molten metal at a temperature lower than 750°C.

In addition, it is preferable that the step of inputting the raw materials of Ca and Y, the master alloy ingot, which contains Mg, Al, Zn, Ca and Y, or the Ca compound and the Y compound into the magnesium alloy molten metal further include the step of periodically stirring the magnesium alloy molten metal.

Furthermore, it is preferable that the casting method be one selected from the group consisting of mold casting, sand casting, gravity casting, squeeze casting, continuous casting, strip casting, die casting, precision casting, lost foam casting, spray casting, and semi-solid casting.

In addition, it is preferable that the method further include the step of carrying out hot working on the magnesium alloy cast material produced by the casting method.

The reasons why the content of respective components in the magnesium alloy of the present invention is limited are as follows.

### Aluminum (Al)

Al is an element that increases the strength, flowability and solidification range of a magnesium alloy, thereby improving castability. In general, the fraction of the eutectic phase increases in response to an increase in the content of Al that is added. In addition, as will be described later, according to the results of experiments of the present invention, it can be appreciated that the ignition resistance increases in response to an increase in the content of Al when Al is added in combination with other alloying elements. When the content of Al is less than 1wt%, the effect of the increased strength and ignition resistance does not occur, and when the content of Al is equal to or greater than 7wt%, tensile properties are degraded due to a coarse Mg₁₇Al₁₂ eutectic phase. Therefore, it is preferred that Al is contained in the range equal to or greater than 1wt% and less than 7wt%.

### Calcium (Ca)

Ca improves the strength and thermal resistance properties of a Mg-Al-based alloy by forming an intermetallic compound as well as reducing the oxidation of a molten metal by forming a thin and dense oxide layer of CaO on the surface of the molten metal, thereby improving the ignition resistance of the Mg alloy. However, when the content of Ca is less than 0.05wt%, the effect of the improved ignition resistance is not significant. On the other hand, when the content of Ca is greater than 2wt%, the castability of the molten metal decreases, hot cracking occurs, die sticking increases, and elongation significantly decreases, which are problematic. Therefore, in the Mg alloy of the present invention, Ca is added in an amount ranging from 0.2wt% to 2.0wt%, and more preferably from 0.2wt% to 1.5wt%.

### Yttrium (Y)

Y is generally used as an element that increases high-temperature creep resistance due to precipitation strengthening, since it has a high solubility limit. When Y is added in combination with Ca to the magnesium alloy, the fraction of the coarse Ca-containing eutectic phase decreases. When Y is added in an amount of 0.05wt% or greater, there is an effect in that AI2Y particles, which form microscopic grains of a cast material, are formed, thereby improving tensile properties. In addition, an oxide layer of Y₂O₃ is formed on the surface of a molten metal to form a mixed layer with MgO and CaO, thereby increasing ignition resistance. When Y is contained in an amount of less than 0.05wt% in the Mg alloy, the increase in the ignition temperature is not significant. When Y is contained in an amount greater than 2wt%, the price of the Mg alloy rises, and the effect of micronization is lost due to the coarsening of Al₂Y particles. Therefore, in the Mg alloy of the present invention, Y is included in an amount ranging from 0.05wt% to 2.0wt%, and more preferably from 0.1wt% to 1.5wt%.

### Zinc (Zn)

Zn has an effect of refining grains and increasing strength when added together with Al. In addition, the maximum solubility limit of Zn in the Mg alloy is 6.2wt%. When an amount of Zn greater than this limit is added, a coarse eutectic phase that is created during casting weakens the mechanical properties of the cast material, and a considerable amount of coarse eutectic phase resides even after homogenization heat treatment, thereby becoming a factor that weakens the mechanical properties, in particular, elongation. Therefore, it is preferred that Zn be added in an amount greater than 0% and equal to or less than 6wt%.

### Manganese (Mn)

In the Mg-Al-based alloy, Mn improves corrosion resistance due to its bonding with Fe, which is an impurity element that impedes corrosion resistance, and increases strength by forming an Al-Mn intermetallic compound at a rapid cooling speed. However, when Mn is added in an amount greater than 1.0wt%, a coarse β-Mn or Al₈Mn₅ phase is formed in the Mg alloy, thereby deteriorating the mechanical properties. Therefore, Mn is included in an amount greater than 0% and equal to or less than 1.0wt%.

### Zirconium (Zr)

Zr is generally added for the purpose of micronization of grains due to the nonhomogeneous nucleation of Mg crystals in primary Zr because the primary Zr, the crystal lattice of which is very similar to Mg crystals, is created during solidification when Zr is added to a Mg alloy that does not contains some elements, such as Al and Mn. When Zr is added in an amount less than 0.1wt%, its effect is not sufficient. When Zr is added in an amount that is greater than 1.0wt%, elongation decreases due to the formation of the coarse primary Zr. Therefore, it is preferred that Zr be added in an amount ranging from 0.1wt% to 1.0wt%.

### Other Unavoidable Impurities

The Mg alloy of the present invention may contain impurities that are unavoidably mixed from raw materials thereof or during the process of manufacture. Among the impurities that can be contained in the Mg alloy of the invention, iron (Fe), silicon (Si) and nickel (Ni) are components that particularly worsen the corrosion resistance of the Mg alloy. Therefore, it is preferred that the content of Fe be maintained at 0.004wt% or less, the content of Si be maintained at 0.04wt% or less, and the content of Ni be maintained at 0.001wt% or less.

### Total Amount of Ca and Y

When Ca and Y are added in combination, a dense combined oxide layer of CaO/Y₂O₃ is formed on the surface of a solid or liquid Mg alloy, so that the ignition resistance of the Mg alloy is superior to that of a Mg alloy to which Ca or Y is separately added. In addition, when Ca or Y is separately added, an amount of 3wt% or greater is generally added in order to obtain excellent ignition resistance. In this case, however, there is a problem in that the tensile properties are greatly degraded because a coarse intermetallic compound is formed. In contrast, the addition of Ca and Y in combination can advantageously improve tensile properties by decreasing the fraction and size of the intermetallic compound while obtaining excellent ignition resistance. When Ca and Y are added to the Mg alloy such that the total content thereof is less than 0.1wt%, the effect of the combined addition of Ca and Y does not appear. This results in a low ignition temperature of 650°C, thereby making it impossible to perform melting in the air or a common inert gas atmosphere. In addition, when the total content of Ca and Y is 2.5wt% or greater, an increase in the cost of the alloy results without any significant advantage related to the additional increase in the ignition temperature. Therefore, in the Mg alloy of the invention, the total content of Ca and Y that are added is in the range from 0.2wt% to 2.0wt%.

### [Advantageous Effects]

The Mg alloy according to the invention forms a dense composite oxide layer that acts as a protective film. Thus the Mg alloy has very excellent oxidation and ignition resistance, can be melted, cast and machined in the air or a common inert atmosphere (Ar or N₂), and can reduce the spontaneous ignition of chips that are accumulated during the process of machining.

In addition, the Mg alloy according to the invention is adapted to reduce costs, protect the health of workers, and prevent environmental pollution since it does not use a protective gas such as SF₆.

Furthermore, the Mg alloy according to the invention is applicable as a material for structural components, since its ignition resistance is superior to that of common alloys, with the ignition temperature thereof being 50°C higher than the melting point thereof, and it also has excellent strength and ductility.

Moreover, the Mg alloy according to the invention can be variously used as a processing material or a cast material, and in particular, can be manufactured as an extruded material, a sheet material, a forged material, a cast material, and the like, which can be practically applied to next-generation vehicles, high-speed rail systems, and the like, in which high-strength, high-elongation and safety characteristics are required.

### [Description of Drawings]

FIG. 1 (a) is a picture showing the surface of an alloy cast material according to comparative example 1, which is manufactured in the air according to an exemplary embodiment of the invention;
FIG. 1 (b) is a picture showing the surface of an alloy cast material according to comparative example 2, which is manufactured in the air according to an exemplary embodiment of the invention;
FIG. 2 is a view illustrating a method of measuring the ignition temperature of a magnesium alloy, which is manufactured according to an exemplary embodiment of the invention;
FIG. 3 is a view showing the results of electron probe micro-analysis (EPMA) on an oxide layer on the surface of a molten metal after a magnesium alloy according to Reference example 5, which was cast according to an exemplary embodiment of the invention, was maintained at 670°C for 10 minutes;
FIG. 4 is a view schematically showing the structure of double composite oxide layers formed on the surface of a solid or liquid phase in an alloy in which Ca and Y are added in combination, the double composite oxide layers serving to block the penetration of external oxygen;
FIG. 5 (a) is an optical picture showing the microscopic structure of an alloy of comparative example 3, which is cast according to an exemplary embodiment of the invention;
FIG. 5 (b) is an optical picture showing the microscopic structure of an alloy of Reference example 2, which is cast according to an exemplary embodiment of the invention;
FIG. 6 (a) is an optical picture showing the microscopic structure of an alloy of comparative example 1, which is extruded according to an exemplary embodiment of the invention;
FIG. 6 (b) is an optical picture showing the microscopic structure of an alloy of comparative example 2, which is extruded according to an exemplary embodiment of the invention;
FIG. 6 (c) is an optical picture showing the microscopic structure of an alloy of comparative example 3, which is extruded according to an exemplary embodiment of the invention;
FIG. 6 (d) is an optical picture showing the microscopic structure of an alloy of example 1, which is extruded according to an exemplary embodiment of the invention;
FIG. 7 is a picture showing variation in the ignition temperature depending on the total amount of Ca and Y that is added in the comparative examples and examples, which are manufactured according to an exemplary embodiment of the invention; and
FIG. 8 is a picture showing variations in the value of tensile strength × uniform elongation depending on the total amount of Ca and Y that is added in the comparative examples and examples, which are manufactured according to an exemplary embodiment of the invention.

### [Best Mode]

Reference will now be made in detail to exemplary embodiments of a Mg alloy and a method of manufacturing the same according to the present invention. However, it is to be understood that the following embodiments are illustrative but do not limited the invention.

As the results of studies that were carried out on a thermodynamically calculated alloy design in order to solve the foregoing problem of the related art and realize the object of the invention, the inventors of the invention found that, when Ca and Y are added in combination to a Mg-Al-based alloy or a Mg-AI-Zn-based alloy, as presented in Table 1 below, the fraction of a hard eutectic phase (eutectic phase I) significantly decreases compared to the case in which Ca is added alone, and at the same time, the formation of a AI2Y phase, i.e. particles that form micronized grains, is induced, so that not only ignition resistance but also tensile strength can be improved.

**Table 1**

| | Al₂Y | Eutectic phase I (Al₂Ca, Mg₂Ca) | Eutectic phase II (Mg₁₇CAL₁₂) |
|---|---|---|---|
| Mg-3AI-1Zn-1Ca | - | 2.241 | |
| Mg-3Al-1 Zn-2Ca | - | 3.733 | |
| Mg-3Al-1Zn-1Ca-0.6Y | 0.845 | 2.169 | |
| Mg-6AI-1Zn-1Ca | - | 2.303 | 4.183 |
| Mg-6AI-1Zn-2Ca | - | 4.600 | 1.776 |
| Mg-6Al-1Zn-1Ca-0.6Y | 0.890 | 2.272 | 3.505 |

The inventors of the invention manufactured Mg alloys having a variety of compositions based on the above data. The method of manufacturing a Mg alloy according to an exemplary embodiment of the invention is as follows.

First, raw materials that include Mg (99.9%), Al (99.9%), Zn (99.99%), Ca (99.9%), Y (99.9%) and selectively Mn (99.9%) were prepared, and were then melted. Then, Mg alloy cast materials having the alloy compositions described in inventive examples 1 and 4 and reference examples 2, 3 and 5-17 and comparative example 1 to comparative example 9 in Table 2 below were formed from the raw materials using a gravity casting method. Specifically, the temperature of a molten metal was increased up to a temperature between 850°C and 900°C, so that these elements were completely melted, in order to produce an alloy by directly inputting Ca and Y, which have high melting points of 842°C and 1525°C, respectively, into the molten metal. After that, the molten metal was gradually cooled down to a casting temperature, and then the Mg alloy cast materials were produced by casting the molten metal.

Alternatively, according to an exemplary embodiment of the invention, it is possible to manufacture a Mg alloy by a variety of methods in addition to the method in which casting is performed after a molten metal is formed by simultaneously melting raw materials including Mg (99.9%), Al (99.9%), Zn (99.99%), Ca (99.9%) and Y (99.9%). In an example, it is possible to first form a Mg alloy molten metal using the raw materials of Mg, Al and Zn or alloys thereof, input the raw materials of Ca and Y, or a Ca compound and a Y compound into the Mg alloy molten metal, and then produce a Mg alloy cast material by a suitable casting method. It is also possible to produce a Mg alloy cast material by preparing a Mg, Al, Zn, Ca and Y alloy (master alloy ingot) of which the contents of Ca and Y are higher than final target values, forming a Mg alloy molten metal using raw materials of Mg, Al and Zn or alloys thereof, and then inputting the master alloy ingot into the Mg alloy molten metal. This method is particularly advantageous in that the master alloy ingot can be input at a temperature that is lower than the temperature at which the raw materials of Ca and Y are directly input into the Mg alloy molten metal, since the melting point of the master alloy ingot is lower than those of the raw materials of Ca and Y. In addition, the formation of a Mg alloy according to the invention can be realized by a variety of methods, and all methods of forming a Mg alloy that are well-known in the art to which the invention belongs are included as part of the invention.

In this embodiment, a graphite crucible was used for induction melting, and a mixture gas of SF₆ and CO₂ was applied on the upper portion of the molten metal, so that the molten metal did not come into contact with the air, in order to prevent the molten metal from being oxidized before the alloying process was finished. In addition, after the melting was completed, mold casting was performed using a steel mold without a protective gas. A sheet-shaped cast material having a width of 100mm, a length of 150mm and a thickness of 15mm was manufactured for a rolling test, a cylindrical billet having a diameter of 80mm and a length of 150mm was manufactured for an extrusion test, and a cylindrical billet having a diameter of 55mm and a length of 100mm was manufactured for an ignition test of the alloy cast material. Although the Mg alloy was cast by a mold casting method in this embodiment, a variety of casting methods, such as sand casting, gravity casting, squeeze casting, continuous casting, strip casting, die casting, precision casting, spray casting, semi-solid casting, and the like, may also be used. Although the Mg alloy according to the invention is not necessarily limited to a specific casting method, fusion casting is more preferable.

Afterwards, the slabs that were prepared above were subjected to homogenization heat treatment at 400°C for 15 hours. In sequence, the materials of comparative example 1 to comparative example 6 and example 1 to example 7 in Table 2, which were subjected to homogenization heat treatment, were machined into sheet materials having a final thickness of 1mm via hot working, in which the respective materials were rolled under conditions of a roll temperature of 200°C, a roll diameter of 210mm, a roll speed of 5.74mpm, and reduction ratios of each roll of 30%/pass and 72%/pass. Here, when the reduction ratio of each roll was 30%/pass, rolling was performed a total of 7 times until the final thickness of 1mm was realized.

In addition, in comparative example 7, comparative example 8 and reference example 8 in Table 2, rod-shaped extruded materials having a final diameter of 16mm were manufactured by extruding the materials that were subjected to homogenization heat treatment under conditions including an extrusion speed of 5m/min, an extrusion ratio of 25:1, and an extrusion temperature of 250. The extruded materials had a good surface state.

Although rolling and extrusion were performed after casting and homogenization heat treatment in this embodiment, the materials may be manufactured by a variety of machining methods, such as forging and drawing, without being necessarily limited to a specific machining method.

### Measurement of Ignition Temperature of Mg Alloy

In order to measure the ignition temperature of the Mg alloys, chips having a predetermined size were produced by machining the outer portion of the cylindrical billets, which were manufactured above, in conditions including a depth of 0.5mm, a pitch of 0.1mm, and a constant speed of 350rpm. 0.1g chips that were produced by the foregoing method were heated by loading them at a constant speed into a heating furnace, which was maintained at 1000°C. The temperatures at which a sudden rise in temperature begins during this process were determined as ignition temperatures, as shown in FIG. 3, and the results are presented in Table 2.

As can be seen from comparative example 1 to comparative example 6 in Table 2, the ignition temperature of Mg alloys suddenly increases in response to the addition of Ca. When the same amount of Ca was added, the ignition temperature of the alloys tends to increase in response to an increase in the content of Al therein.

**Table 2**

| | Alloy Symbol | Alloy Composition (wt%) | | | | | | Ignition Temp (°C) | Test Atm. |
|---|---|---|---|---|---|---|---|---|---|
| | | Al | Zn | Ca | Y | Mn | Zr | | |
| Comp. Ex. 1 | AZ31 | 3 | 1 | | | | | 490 | Air |
| | | | | | | | | 554 | Air + Ar |
| Comp. Ex. 2 | AZX311 | 3 | 1 | 1 | | | | 708 | Air |
| Comp. Ex. 3 | AZX312 | 3 | 1 | 2 | | | | 747 | Air |
| Comp. Ex. 4 | AZ61 | 6 | 1 | | | | | 507 | Air |
| | | | | | | | | 602 | Air + Ar |
| Comp. Ex. 5 | AZX611 | 6 | 1 | 1 | | | | 703 | Air |
| Comp. Ex. 6 | AZX612 | 6 | 1 | 2 | | | | 755 | Air |
| Comp. Ex. 7 | ZX61 | | 6 | 1 | | | | 672 | Air |
| Comp. Ex. 8 | ZX62 | | 6 | 2 | | | | 704 | Air |
| Comp. Ex. 9 | ZK60 | | 5.5 | | | | 0.45 | 553 | Air |
| Inventive Example 1 | Alloy 1 | 3 | 0.8 | 1 | 1 | 0.3 | | 807 | Air |
| Reference Example 2 | Alloy 2 | 3 | 1 | 1 | 0.6 | | | 768 | Air |
| | | | | | | | | 776 | Air + Ar |
| Reference Example 3 | Alloy 3 | 3 | 1 | 0.7 | 0.6 | | | 714 | Air |
| | | | | | | | | 707 | Air + Ar |
| Inventive Example 4 | Alloy 4 | 3 | 0.8 | 0.3 | 0.3 | 0.25 | | 698 | Air |
| | | | | | | | | 705 | Air + Ar |
| Reference Example 5 | Alloy 5 | 6 | 1 | 1 | 0.6 | | | 774 | Air |
| Reference Example 6 | Alloy 6 | 6 | 1 | 0.7 | 0.6 | | | 745 | Air |
| | | | | | | | | 749 | Air + Ar |
| Reference Example 7 | Alloy 7 | 6 | 1 | 0.3 | 0.3 | | | 705 | Air |
| | | | | | | | | 717 | Air + Ar |
| Reference Example 8 | Alloy 8 | 6 | 1 | 0.1 | 0.1 | | | 677 | Air |
| Reference Example 9 | Alloy 9 | 6 | 2 | 1 | 0.6 | | | 783 | Air |
| Reference Example 10 | Alloy 10 | 6 | 2 | 0.1 | 0.1 | | | 658 | Air |
| | | | | | | | | 711 | Air + Ar |
| Reference Example 11 | Alloy 11 | 4 | 4 | 0.7 | 0.6 | | | 771 | Air |
| Reference Example 12 | Alloy 12 | 4 | 4 | 0.1 | 0.1 | | | 653 | Air |
| | | | | | | | | 676 | Air + Ar |
| Reference Example 13 | Alloy 13 | 1 | 6 | 1 | 1 | | | 744 | Air |
| Reference Example 14 | Alloy 14 | 1 | 6 | 0.7 | 0.6 | | | 689 | Air |
| Reference Example 15 | Alloy 15 | 1 | 6 | 1 | 0.3 | | | 659 | Air |
| Reference Example 16 | Alloy 16 | 2 | 6 | 1 | 1 | | | 755 | Air |
| Reference Example 17 | Alloy 17 | 1 | 6 | 0.7 | 0.6 | | 0.2 | 698 | Air |

In Table 2, showing inventive examples 1 and 4 and reference examples 2, 3 and 5-17 comparing each ignition temperature of reference example 2 and reference example 5 with the respective ignition temperature of comparative reference example 2 and comparative example 5, it can be appreciated that the ignition temperature is much higher when Y was also added to the Mg alloys than when Ca was added alone to the Mg alloys. This is because a mixed layer of CaO and Y₂O₃ was formed in the portion that was in contact with molten metal due to the addition of Y, as can be seen from the result of electron probe micro-analysis (EPMA) of FIG. 4, and that this layer was able to effectively reduce the oxygen in the air from penetrating into and reacting with the molten metal. In addition, a mixed layer of CaO and MgO was present in the outer portion of the mixed layer of CaO and Y₂O₃. These double mixed layers help the molten metal remain stable even at high temperatures.

In addition, comparing comparative example 3 with reference example 2 and comparative example 6 with reference example 5, it can be appreciated that the ignition temperature was higher when Ca and Y were added in combination than when Ca was added alone, even though the total content of Ca and Y was less than the content of Ca. This shows that a more excellent effect can be realized in terms of increasing ignition resistance when Ca and Y are added in combination than when Ca is used alone in order to increase the ignition temperature of the Mg alloy.

In addition, Table 2 presents that the Mg alloy according to inventive example 1 has a very high ignition temperature of 807°C. This is because Y has a very high content of 1wt%. Thus, it can be appreciated that ignition resistance can significantly increase in response to an increase in the content of Y that is added. Furthermore, in Table 2, the Mg alloy according to reference example 8 has a very high ignition resistance of 811°C. This shows that the ignition temperature of the Mg alloy, in which 6wt% of Zn is added, significantly increases when Ca and Y are added respectively in an amount of 1wt%.

### Evaluation of Tensile Properties of Mg Alloy

The sheet materials, which were manufactured by the above-described method, were heat-treated at 250°C for 30 minutes, and then sub-size sheet-shaped samples according to the ASTM-E-8M standard, in which the length of a gauge was 25mm, were produced. A tensile test was carried out at room temperature under a strain of 1 × 10⁻³s⁻¹ using a common tensile tester, and the results are presented in Table 3.

In addition, samples of a rod-shaped extruded material, in which the length of a gauge was 25mm, were manufactured, and tensile test was carried out under the same conditions as for the sheet-shaped samples.

As presented in Table 3, comparing comparative example 2 with comparative example 3, comparative example 5 with comparative example 6, and comparative example 7 with comparative example 8, it can be appreciated that the yield strength and tensile strength increased but elongation significantly decreased in response to the increase in the content of Ca from 1wt% to 2wt%. This decrease in the elongation is because the fraction of a microscopic precipitate phase of Al₂Ca as well as the fraction of a coarse and hard ternary eutectic phase of Mg-Al-Ca increased, as shown in FIG. 5 (a), when the content of Ca that was added was increased to 2wt%. In contrast, as shown in FIG. 5 (b), when the content of Ca that was added was 1wt%, even though 0.6wt% of Y was included, no coarse and hard ternary eutectic phase of Mg-Al-Ca was observed and thus elongation was not decreased. Likewise, comparing the microscopic structures of the extruded materials of comparative example 1 to comparative example 3 and inventive example 1 with reference to FIG. 6, when the content of Ca that was added was increased to 1wt% and 2wt%, large amounts of black second phases, indicated by the arrows in FIG. 6 (b) and FIG. 6 (c), respectively, were observed, and elongation decreased since the hard second phases were vulnerable to defects.

**Table 3**

| | Alloy Symbol | Tensile Properties | | | | | |
|---|---|---|---|---|---|---|---|
| | | YS¹⁾ (MPa) | TS²⁾ (MPa) | EI³⁾ (%) | UEI⁴⁾ (%) | TS X UEI (MPa●%) | Remarks |
| Comp. Ex. 1 | AZ31 | 176.4 | 274.5 | 25.2 | 17.4 | 4788 | RAM⁵⁾ |
| | | 176.8 | 270.4 | 26.0 | 15.3 | 4142 | EM⁶⁾ |
| Comp. Ex. 2 | AZX311 | 191.1 | 276.1 | 24.3 | 16.9 | 4658 | RAM |
| | | 239.4 | 294.5 | 17.1 | 11.8 | 3479 | EM |
| Comp. Ex. 3 | AZX312 | 255.2 | 303.6 | 16.5 | 9.7 | 2943 | RAM |
| | | 346.0 | 355.4 | 9.0 | 5.8 | 2045 | EM |
| Comp. Ex. 4 | AZ61 | 218.7 | 324.0 | 22.0 | 17.2 | 5565 | RAM |
| | | 166.5 | 298.1 | 26.4 | 21.1 | 6292 | EM |
| Comp. Ex. 5 | AZX611 | 204.4 | 306.2 | 19.7 | 16.0 | 4909 | RAM |
| | | 150.8 | 276.9 | 21.2 | 19.3 | 5337 | EM |
| Comp. Ex. 6 | AZX612 | 230.0 | 321.0 | 16.7 | 14.1 | 4536 | RAM |
| | | 169.9 | 275.6 | 19.2 | 16.4 | 4533 | EM |
| Comp. Ex. 7 | ZX61-F | 191.4 | 268.1 | 25.4 | 17.2 | 4606 | EM |
| Comp. Ex. 8 | ZX62-F | 294.9 | 298.5 | 13.7 | 9.4 | 2791 | EM |
| Comp. Ex. 9 | ZK60-F | 238.4 | 318.4 | 24.1 | 13.5 | 4298 | EM |
| Reference Example 2 | Alloy 2 | 175.8 | 265.2 | 24.7 | 18.4 | 4880 | RAM |
| Reference Example 3 | Alloy 3 | 171.1 | 264.3 | 26.5 | 18.4 | 4856 | RAM |
| Inventive Example 4 | Alloy 4 | 175.1 | 267.4 | 27.8 | 16.8 | 4483 | EM |
| Reference Example 5 | Alloy 5 | 225.7 | 323.4 | 19.6 | 15.5 | 5020 | RAM |
| Reference Example 8 | Alloy 8 | 156.3 | 297.6 | 26.8 | 22.6 | 6738 | EM |
| Reference Example 9 | Alloy 9 | 242.1 | 337.0 | 16.8 | 15.3 | 5157 | RAM |
| Reference Example 10 | Alloy 10 | 215.1 | 340.2 | 21.7 | 19.5 | 6633 | EM |
| Reference Example 11 | Alloy 11 | 152.0 | 302.1 | 33.5 | 29.1 | 8780 | EM |
| Reference Example 12 | Alloy 12 | 189.8 | 323.7 | 27.3 | 22.7 | 7338 | EM |
| Reference Example 13 | Alloy 13 | 161.5 | 276.1 | 26.8 | 22.4 | 6196 | RAM |
| Reference Example 14 | Alloy 14 | 165.9 | 288.3 | 30.3 | 25.9 | 7467 | EM |
| Reference Example 15 | Alloy 15 | 167.5 | 280.8 | 31.3 | 23.9 | 6711 | EM |
| Reference Example 16 | Alloy 16 | 175.3 | 285.7 | 26.5 | 22.3 | 6363 | EM |

| | | | | | | | |
|---|---|---|---|---|---|---|---|
| Notes) YS¹⁾: Yield Strength, TS²⁾: Tensile Strength, EI³⁾: Elongation, UEI⁴⁾: Uniform Elongation, RAM⁵⁾: Rolled and Annealed Material, EM⁶⁾: Extruded Material | | | | | | | |

On the other hand, as shown in FIG. 6 (d), no hard second phase that decreases elongation was observed in the extruded material of an alloy in which each of Ca and Y was added in an amount of 1wt%. This result is more apparent when comparing reference example 2 with comparative example 3, reference example 5 with comparative example 6, and reference example 13 with comparative example 8. Specifically, it can be appreciated that, even though only 1wt% of Ca and 0.6wt% of Y were added in reference example 2 and reference example 5, their elongation was very high and their ignition resistance and tensile strength were at levels similar to those of comparative example 3 and comparative example 6, in which 2wt% of Ca was added. Likewise, in reference example 13, it can be appreciated that the ignition resistance was greatly increased and that the tensile properties, particularly the value of tensile strength × uniform elongation, were greatly increased when 1wt% of Ca and 1wt% of Y were added to the Mg-6Zn-1Al alloy. That is, due to the addition of a small amount of Y, it was possible to produce a Mg alloy of this embodiment in which the content of Ca was maintained low, on the order of 1wt%, but in which the fraction of the coarse and hard ternary eutectic phase was greatly decreased, such that both strength and elongation were improved.

In addition, comparing reference example 2 with comparative example 2 and reference example 5 with comparative example 5, it can be appreciated that reference example 2 and reference example 5 contain the same content of Ca that was added in relation to the addition of Y, and have ignition resistance that is superior to that of the case in which Y was not added. At the same time, the value of tensile strength × uniform elongation is further increased.

This tendency can be appreciated from FIG. 7 and FIG. 8, which show variations in the ignition temperature and tensile properties thereof in response to the total amount of Ca and Y that was added. As shown in FIG. 7, the ignition temperature tends to gradually increase in response to an increase in the total amount of Ca and Y that was added. In particular, it can be appreciated that the slope of the increase in the ignition temperature is further increased when Y is added than when Y is not added. In contrast, as shown in FIG. 8, when Ca is added alone, the value of tensile strength × uniform elongation tends to greatly decrease in response to an increase in the content of Ca that is added, irrespective of the type of hot working. However, when both Ca and Y are added, the mechanical strength thereof is improved more than that of an alloy in which neither Ca nor Y is added. From these results, it can be appreciated that the ignition resistance is greatly increased, and at the same time that tensile properties are greatly improved due to the addition of a small content of Ca and Y at the same time.

The Mg alloy and the method of manufacturing the same according to exemplary embodiments of the present invention have been described above in detail with reference to the accompanying drawings. However, it will be apparent to a person having ordinary skilled in the art to which the present invention belongs that the foregoing embodiments are merely examples of the invention and various modifications and variations are possible. Therefore, it should be understood that the scope of the invention shall be defined only by the appended claims.

## Claims

1. A magnesium alloy manufactured by melt casting, the magnesium alloy comprising, by weight, 1.0% or greater but less than 7.0% of Al, 0.2% to 2.0% of Ca, 0.05% to 2.0% of Y, greater than 0% to 6% of Zn, greater than 0% to 1% of Mn, optionally 0.1 % to 1.0% of Zr, a balance of Mg, and other unavoidable impurities, wherein a total content of the Ca and the Y is equal to or greater than 0.2% but less or equal than 2.0% of a total weight of the magnesium alloy and
wherein a combined oxide layer of CaO/Y₂O₃ is formed on the surface of the magnesium alloy.

2. The magnesium alloy of claim 1, wherein a content of the Ca ranges, by weight, from 0.2% to 1.5%.

3. The magnesium alloy of claim 1, wherein a content of the Y ranges, by weight, from 0.1 % to 1.5%.

4. The magnesium alloy of any one of claims 1 to 3, wherein contents of the Ca and the Y range from 0.3% to 2.0% of a total weight of the magnesium alloy.

5. A method of manufacturing a magnesium alloy, comprising:
forming a magnesium alloy molten metal, which contains Mg, Al and Zn;
adding raw materials of Ca and Y into the magnesium alloy molten metal;
producing a magnesium alloy cast material from the magnesium alloy molten metal, in which the raw materials of Ca and Y are added, using a fusion casting method,
wherein a magnesium alloy, which is produced by the above process, comprises, by weight, 1.0% or greater but less than 7.0% of Al, 0.2% to 2.0% of Ca, 0.05% to 2.0% of Y, greater than 0% to 6% of Zn, greater than 0% to 1% of Mn, optionally 0.1 % to 1.0% of Zr, a balance of Mg, and other unavoidable impurities,
wherein a total content of the Ca and the Y is equal to or greater than 0.2 % but less or equal than 2.0% of a total weight of the magnesium alloy, and
wherein a combined oxide layer of CaO/Y₂O₃ is formed on the surface of the magnesium alloy.

6. The method of claim 5, wherein adding the raw materials of Ca and Y into the magnesium alloy molten metal comprises adding the raw materials of Ca and Y at a temperature higher than 800°C.

7. The method of claim 5 adding raw materials of Ca and Y comprises forming a master alloy ingot, which contains Mg, Al, Zn, Ca and Y, and is soluble at 750°C or lower.

8. The method of claim 7, wherein the master alloy ingot, which contains Mg, Al, Zn, Ca and Y, is soluble at 750°C or lower, and is input into the magnesium alloy molten metal at a temperature lower than 750°C.

9. The method of claim 5,
the raw materials of Ca is a Ca compound and the raw materials of Y is a Y compound.

10. The method of any one of claims 5 to 9, wherein inputting the raw materials of Ca and Y, the master alloy ingot,
which contains Mg, Al, Zn, Ca and Y, or the Ca compound and the Y compound into the magnesium alloy molten metal further comprises periodically stirring the magnesium alloy molten metal.

11. The method of any one of claims 5 to 9, wherein the casting method comprises one selected from the group consisting of mold casting, sand casting, gravity casting, squeeze casting, continuous casting, strip casting, die casting, precision casting, lost foam casting, spray casting, and semi-solid casting.

12. The method of any one of claims 5 to 9, further comprising carrying out hot working on the magnesium alloy cast material produced by the casting method.

## Patentansprüche

1. Eine Magnesiumlegierung, die durch ein Schmelzgießen hergestellt wird, wobei die Magnesiumlegierung gewichtsmäßig 1% oder mehr, aber weniger als 7,0% Al, 0,2% bis 2,0% Ca, 0,05% bis 2,0% Y, mehr als 0% bis 6% Zn, mehr als 0% bis 1% Mn, optional 0,1% bis 1,0% Zr, einen Ausgleich an Mg und andere unvermeidbare Verunreinigungen aufweist,
wobei ein Gesamtgehalt des Ca und Y gleich oder größer als 0,2%, aber geringer als oder gleich 2,0% des Gesamtgewichts der Magnesiumlegierung ist und
wobei eine kombinierte Oxidschicht aus CaO/Y₂O₃ auf der Oberfläche der Magnesiumlegierung gebildet ist.

2. Die Magnesiumlegierung nach Anspruch 1, wobei sich ein Gehalt des Ca gewichtsmäßig von 0,2% bis 1,5% bewegt.

3. Die Magnesiumlegierung nach Anspruch 1, wobei sich ein Gehalt des Y gewichtsmäßig von 0,1% bis 1,5% bewegt.

4. Die Magnesiumlegierung nach einem der Ansprüche 1 bis 3, wobei sich Gehalte des Ca und des Y von 0,3% bis 2,0% eines Gesamtgewichts der Magnesiumlegierung bewegen.

5. Ein Verfahren zum Herstellen einer Magnesiumlegierung, umfassend:
Bilden eines geschmolzenen Metalls aus einer Magnesiumlegierung, die Mg, Al und Zn enthält;
Zufügen von Rohmaterialien aus Ca und Y in das geschmolzene Metall aus einer Magnesiumlegierung;
Erzeugen eines Gussmaterials aus einer Magnesiumlegierung aus dem geschmolzenen Metall einer Magnesiumlegierung, in das die Rohmaterialien aus Ca und Y hinzugefügt sind, unter Verwendung eines Schmelzgussverfahrens,
wobei eine Magnesiumlegierung, die durch das obige Verfahren hergestellt ist, gewichtsmäßig 1% oder mehr, aber weniger als 7,0% Al, 0,2% bis 2,0% Ca, 0,05% bis 2,0% Y, mehr als 0% bis 6% Zn, mehr als 0% bis 1% Mn, optional 0,1% bis 1,0% Zr, einen Ausgleich an Mg und andere unvermeidbare Verunreinigungen aufweist,
wobei ein Gesamtgehalt des Ca und Y gleich oder größer als 0,2%, aber geringer als oder gleich 2,0% des Gesamtgewichts der Magnesiumlegierung ist und
wobei eine kombinierte Oxidschicht aus CaO/Y₂O₃ auf der Oberfläche der Magnesiumlegierung gebildet ist.

6. Das Verfahren nach Anspruch 5, wobei das Zufügen der Rohmaterialien aus Ca und Y in das geschmolzene Metall aus einer Magnesiumlegierung ein Zufügen der Rohmaterialien aus Ca und Y bei einer höheren Temperatur als 800°C umfasst.

7. Das Verfahren nach Anspruch 5, wobei das Zufügen der Rohmaterialien aus Ca und Y ein Bilden eines Masterlegierungsblocks umfasst, der Mg, Al, Zn, Ca und Y enthält und bei 750°C oder weniger löslich ist.

8. Das Verfahren nach Anspruch 7, wobei der Masterlegierungsblock, der Mg, Al, Zn, Ca und Y enthält, bei 750°C oder weniger löslich ist und bei einer Temperatur unterhalb von 750°C in das geschmolzene Metall aus einer Magnesiumlegierung eingebracht wird.

9. Das Verfahren nach Anspruch 5, wobei das Rohmaterial aus Ca eine Ca-Verbindung ist und das Rohmaterial aus Y eine Y-Verbindung ist.

10. Das Verfahren nach einem der Ansprüche 5 bis 9, wobei das Einfügen der Rohmaterialien aus Ca und Y, des Masterlegierungsblocks, der Mg, Al, Zn, Ca und Y enthält, oder der Ca-Verbindung und der Y-Verbindung in das geschmolzene Metall aus einer Magnesiumlegierung weiterhin ein periodisches Rühren des geschmolzenen Metalls aus einer Magnesiumlegierung umfasst.

11. Das Verfahren nach einem der Ansprüche 5 bis 9, wobei das Gießverfahren eines umfasst, das aus der Gruppe ausgewählt ist, die aus Formgießen, Sandgießen, Schwerkraftgießen, Squeezegießen, Stranggießen, Stripgießen, Spritzgießen, Präzisionsgießen, Vollformgießen, Spraygießen und Semi-Solid-Gießen besteht.

12. Das Verfahren nach einem der Ansprüche 5 bis 9, weiter umfassend ein Durchführen eines Warmbearbeitens des Gussmaterials aus einer Magnesiumlegierung, das durch das Gießverfahren hergestellt ist.

## Revendications

1. Alliage de magnésium fabriqué par coulée d'une masse fondue, l'alliage de magnésium comprenant, en poids, 1,0 % ou plus mais moins de 7,0 % d'AI, de 0,2 % à 2,0 % de Ca, de 0,05 % à 2,0 % de Y, de plus de 0 % à 6 % de Zn, de plus de 0 % à 1 % de Mn, facultativement de 0,1 % à 1,0 % de Zr, le reste étant constitué de Mg et d'autres impuretés inévitables,
dans lequel une teneur totale du Ca et de l'Y est supérieure ou égale à 0,2 % mais inférieure ou égale à 2,0 % d'un poids total de l'alliage de magnésium et
dans lequel une couche d'oxydes combinés de CaO/Y₂O₃ est formée sur la surface de l'alliage de magnésium.

2. Alliage de magnésium selon la revendication 1, dans lequel une teneur du Ca se situe dans la plage, en poids, de 0,2 % à 1,5 %.

3. Alliage de magnésium selon la revendication 1, dans lequel une teneur de l'Y se situe dans la plage, en poids, de 0,1 % à 1,5 %.

4. Alliage de magnésium selon l'une quelconque des revendications 1 à 3, dans lequel les teneurs du Ca et de l'Y se situent dans la plage de 0,3 % à 2,0 % d'un poids total de l'alliage de magnésium.

5. Procédé de fabrication d'un alliage de magnésium, comprenant:
la formation d'un métal fondu d'alliage de magnésium, qui contient du Mg, de l'Al et du Zn ;
l'ajout de matériaux bruts de Ca et d'Y dans le métal fondu d'alliage de magnésium ;
la production d'un matériau coulé d'alliage de magnésium à partir du métal fondu d'alliage de magnésium, dans lequel les matériaux bruts de Ca et d'Y sont ajoutés, en utilisant un procédé de coulée par fusion,
dans lequel un alliage de magnésium, qui est produit par le procédé ci-dessus, comprend, en poids, 1,0 % ou plus mais moins de 7,0 % d'AI, de 0,2 % à 2,0 % de Ca, de 0,05 % à 2,0 % de Y, plus de 0 % à 6 % de Zn, plus de 0 % à 1 % de Mn, facultativement de 0,1 % à 1,0 % de Zr, le reste étant constitué de Mg et d'autres impuretés inévitables,
dans lequel une teneur totale du Ca et de l'Y est supérieure ou égale à 0,2 % mais inférieure ou égale à 2,0 % d'un poids total de l'alliage de magnésium, et
dans lequel une couche d'oxydes combinés de CaO/Y₂O₃ est formée sur la surface de l'alliage de magnésium.

6. Procédé selon la revendication 5, dans lequel l'ajout des matériaux bruts de Ca et d'Y dans le métal fondu d'alliage de magnésium comprend l'ajout des matériaux bruts de Ca et d'Y à une température supérieure à 800 °C.

7. Procédé selon la revendication 5, l'ajout de matériaux bruts de Ca et d'Y comprend la formation d'un lingot d'alliage mère, qui contient du Mg, de l'Al, du Zn, du Ca et de l'Y, et est soluble à 750 °C ou moins.

8. Procédé selon la revendication 7, dans lequel le lingot d'alliage mère, qui contient du Mg, de l'Al, du Zn, du Ca et de l'Y, est soluble à 750 °C ou moins, et est introduit dans le métal fondu d'alliage de magnésium à une température inférieure à 750 °C.

9. Procédé selon la revendication 5,
les matériaux bruts de Ca sont constitués d'un composé de Ca et les matériaux bruts d'Y sont constitués d'un composé d'Y.

10. Procédé selon l'une quelconque des revendications 5 à 9, dans lequel l'introduction des matériaux bruts de Ca et d'Y, le lingot d'alliage mère,
qui contient du Mg, de l'Al, du Zn, du Ca et de l'Y, ou le composé de Ca et le composé d'Y dans le métal fondu d'alliage de magnésium, comprend en outre l'agitation périodique du métal fondu d'alliage de magnésium.

11. Procédé selon l'une quelconque des revendications 5 à 9, dans lequel le procédé de coulée comprend l'un choisi dans le groupe constitué d'une coulée en moules, d'une coulée en sable, d'une coulée par gravité, d'une coulée sous pression, d'une coulée continue, d'une coulée en bande, d'une coulée mécanique, d'une coulée de précision, d'une coulée à mousse perdue, d'une coulée par projection et d'une coulée semi-solide.

12. Procédé selon l'une quelconque des revendications 5 à 9, comprenant en outre la réalisation d'un formage à chaud sur le matériau coulé d'alliage de magnésium produit par le procédé de coulée.
